

## UNITED STATES PATENT OFFICE

RICHARD R. WALTER, OF STARNBERG, GERMANY

## PROCESS FOR PRODUCING SINTERED ALLOYS

no Drawing. Application filed December 4, 1930, Serial No. 499,980, and in Germany January 4, 1930.

My invention relates to a process advantageously applicable in the manufacture of sintered metal bodies.

Articles produced from powdered metals or metallic combinations with the aid of pressing and sintering, frequently require a machining operation like sawing, grinding or drilling in order to produce their final form prior to becoming sintered. In most cases the compression is of itself inadequate to attain the required mechanical cohesion. Consequently, such articles have hitherto been presintered, which is to say preheated to about a red glow.

That method of enhancing cohesion is cumbersome and requires special furnaces. Moreover it has the drawback attending the fact that most of the metals or their metallic combinations like the carbides, nitrides and others react more or less with the furnace gases while so glowing and can suffer changes leastways superficially in their structure.

According to the present invention, the articles are strengthened after compression and while cold, by utilization of the binding action of vegetable oils which contain unsaturated fatty acids. Such oils which contain the glycerides of linol, linoleum, isolinoleum of fatty acid are mixed in small percentages with the metal powders before they become pressed; care being taken that a completely uniform distribution occurs, the accomplishment of which is favored if the metal powders are not entirely dry, instead, manifest a moisture of about one to two per cent.

After pressing the articles, atmospheric oxygen causes an oxidation and polymerization of the unsaturated acids whereupon they stiffen completely in a few hours. The oxidation can be curtailed an hour by conducting warmed air of about one to two hundred degrees to the pieces. Thereafter the articles are so hard and edge-secure that one may subject them to every required operation without danger of fracture.

A large number of oils containing unsaturated acids are available for use in this described process for example, sojabean oil, lin-

seed oil, pitch pine oil, Japanese wood oil, and others.

The varnish derivatives of such oils are also capable of application with especial advantage; generally an oil is better for this process in direct proportion as its increased iodine content.

The process may be modified by spraying the oil upon the press-formed pieces, or by effecting an incorporation through a daubing operation; in either case, the absorption-ability of the pieces can be enhanced if the oils are applied with a thin fluid vehicle like benzine or emulsions. This method of impregnation of the articles is less exact than the addition of the oils before pressing.

I claim:

1. The process for producing sintered bodies of powdered metals, comprising, uniformly impregnating a slightly moistened powdered metallic aggregate with a vegetable oil containing unsaturated fatty acids, forming the aggregate by pressing while at atmospheric temperature, allowing it to stiffen by atmospheric exposure whereby to increase the cohesiveness of the formed body and then sintering.

2. The process for producing sintered bodies of powdered metals, comprising, the homogeneous mixing of a vegetable oil having fatty acid and iodine content with powdered metals, forming the mixture by pressing into a body of desired shape, allowing oxidation and polymerization to occur in the presence of warmed air and subsequently sintering.

Signed this 31st day of October, 1930.

RICHARD R. WALTER.